

## UNITED STATES PATENT OFFICE

GEORGES CLAUDE, OF BOULOGNE SUR SEINE, FRANCE, ASSIGNOR TO CLAUDE NEON LIGHTS, INC., OF NEW YORK, N. Y., A CORPORATION OF NEW YORK

## LUMINESCENT TUBE

No Drawing. Application filed June 8, 1929, Serial No. 369,534, and in France August 30, 1928.

This invention relates to gaseous conductor tube lights of the kind in which a column of more or less rarefied gas is rendered luminous by the passage of current between spaced electrodes.

In the production of light by the luminescence of gases or vapors in gaseous conductor tubes difficulty has been experienced in effecting the simultaneous vibration of two or more kinds of atoms. Almost invariably the operating conditions which are realized tend to favor the vibration of one kind of atom and dampen the vibrations of the other kind. One of the most striking examples of this phenomena arises when a mixture of neon gas and mercury vapor in a tube having capillary portions is subjected to a current. The spectrum of mercury is attained in the portions of greater diameter, while in the narrower portions only the spectrum of neon is visible. Similarly, the vibration of nitrogen or hydrogen atoms in a tube of constant diameter containing a mixture of neon with only a few thousandths parts of nitrogen or hydrogen masks the neon spectrum.

The object of the present invention is a luminous tube containing a plurality of gases and wherein the vibration of the atoms of the gaseous contents are not damped but light from all the gases blend to produce a light of pleasing appearance. More particularly, a mixture of helium and neon in a positive column tube light is utilized to produce a very good correction of the wan helium light. For example, if neon is added to the helium in a discharge tube in the proportions, say of one-one hundredth or even one-one thousandth part of neon to one part of helium, when the gaseous contents are ionized, the spectrum of neon appears in a very steady manner and in such a way that the resulting light is neither the light emitted by helium nor that of neon but both blend to produce a very pretty pinkish color which is the more accentuated as the proportion of neon increases. Even when the neon is present in the tube in an amount as small as one-one thousandth part to one part of

helium, the correction of the helium light is noticeable.

The luminous efficiency of such a luminous tube, i. e., the amount of light emitted per watt input, is improved over that of a discharge tube containing only helium, doubtless because the proportion of the total radiation furnished by the neon is attended with the excellent efficiency inherent in this gas for luminescence. The luminous efficiency of the tube is also a function of the pressure of gas in the tube and hence, as the pressure is increased, the intensity of the pinkish color increases, that is, if the pressure of the gaseous contents is increased a lower percentage of neon will give the same luminous efficiency as a higher percentage of neon in a tube wherein the total pressure of the gaseous contents is less. For instance, with a mixture of 0.5% of neon and 99.5% of helium in a tube of 33 millimeters diameter and in which the barometric pressure is 1½ millimeters of mercury, the color of light emitted is of a pale pink color whereas the color is caused to be decidedly darker if the barometric pressure is increased to 3 millimeters of mercury.

It is thus seen that the quality of the light emitted by a gaseous conductor tube and its efficiency is increased by adding to the helium contents a quantity of neon and it has been found that the percentage of neon may vary from less than one one-thousandth part to from 3 to 5% or more and even to 15% according to the effect to be obtained, the diameter of the tube, and the pressure.

Various modifications will occur to those skilled in the art in the gaseous components of the tube and their proportion and the total pressure as well as the character of tube electrodes and no limitation is intended by the phraseology of the foregoing description except as indicated in the appended claims.

What I claim is:—

1. A luminous tube containing one or more of the rare gases including neon, wherein the percentage of neon ranges from 0.001 to 0.15.
2. A luminous tube containing neon and a rare gas wherein the proportion of neon is from less than 0.1 per cent to 15 per cent.

3. A luminous tube containing neon and helium wherein the proportion of neon is from 0.1 per cent to 15 per cent.
4. A luminous tube containing neon and helium in the proportion of 0.5 per cent neon to 99.5 per cent helium.
5. A luminous tube containing neon and helium in the ratio of from less than 0.1 per cent of neon to 3 per cent thereof.
- 10 6. The method of obtaining a blended neon-helium light in which the spectra of both gases are blended which comprises blending neon with helium in the ratio of not over 15 per cent neon and discharging an electric current through the mixture.

In testimony whereof I affix my signature.  
**GEORGES CLAUDE.**

20

25

30

35

40

45

50

55

60

65